

## UNITED STATES PATENT OFFICE

HARRY HINTZE, OF PATERSON, NEW JERSEY

## PROCESS FOR WEIGHTING OF NATURAL AND ARTIFICIAL SILK FIBERS

No Drawing.

Application filed April 22, 1932. Serial No. 607,906.

This invention refers to a process for the weighting of natural and artificial silk fibers with metallic compounds, the term "weighting" in this connection being used to designate the method of increasing the weight and the diameter of the fibers.

In processes heretofore made use of for the weighting of natural silk and other fibers, in the form of skeins and woven or knitted fabrics, a number of chemical substances were brought into contact with the fiber, but all in separate baths, and each containing only one of the necessary weighting or fixing materials. Between each of the baths the silk had to undergo a very thorough rinsing with hard, soft or soured water, depending upon the bath it had passed through last.

In practice the use of metallic compounds such as of iron—for black and navy blue only—alumina, bismuth, zinc, tin and lead has been resorted to; however, a tin-metal solution has proven best.

According to the well-known methods now and heretofore employed, the natural, boiled-off silk is treated first with a solution of tetrachloride of tin— $\text{SnCl}_4 \cdot 5\text{H}_2\text{O}$ —of about 22 degrees Bé. strength at a temperature of 60 degrees F. for some time, and then is rinsed thoroughly with hard water (6 degrees—9 degrees hardness) in order to hydrolyze the tin-metal salt and to precipitate same on the fiber in the form of stannic acid— $\text{H}_2\text{SnO}_4$ . This stannic acid precipitate is then fixed by a treatment of the silk with di-sodium phosphate— $\text{HNa}_2\text{PO}_4 \cdot 12\text{H}_2\text{O}$ —of about 7 degrees Bé. strength at about 60 degrees C. The stannic chloride baths and the phosphate baths are alternately repeated until the desired degree of weighting has been obtained, and after each bath or treatment, the silk has to undergo a water rinsing or neutralization as described above. After the last phosphate bath and subsequent rinsing, a treatment in a solution of sodium silicate— $\text{Na}_2\text{SiO}_4$ —of about 5 Bé. strength and at a temperature of 45° C. is applied.

The silk which has been manipulated in this manner and weighted with complex compounds of tin, phosphate and silicate is then rinsed, soaped and soured and is ready

to be further processed by dyeing and finishing.

The operations described in the foregoing paragraph, as well as other methods of weighting with various substances, are well known and generally practised in the industry at the present time

On account of the tendering effect on the tensile strength of the fiber of too heavy and too many charges of tin-phosphate compounds, and their costs, and the time necessary for the many baths and washings, the weighting process is generally limited to four applications of tin-phosphate and their attendant rinsings, with an average increase in weight of about 11% for each pass and an aggregate gain of about 45% over the weight of the boiled-off silk.

The purpose of the present invention is to improve upon the methods now in use and to provide a process which is shorter, simpler and less expensive and which at the same time produces considerably more weight in natural silk and other fibers, without impairing their tensile strength nor destroying or diminishing their desirable and characteristic qualities.

As is well known in the chemistry of weighting, natural silk charged with metal salts such as iron, alumina, zinc and tin offer a special affinity for lead compounds. By applying lead-metal salts to previously tin-weighted silk, much larger gains in weight per single charge are obtained than those made with other metals. By extensive experiments it was found that the silk-weighting process can be materially simplified and cheapened, when some of the ingredients usually applied in separate baths, namely metal and phosphate compounds, are used in a single bath. The many washings with their necessary losses of materials and the enormous amounts of water can be saved.

In the present invention the silk is treated two or three times in the old and well-known manner with stannic-metal salt and di-sodium phosphate in separate baths, and thorough rinsings after each, and producing a gain of from 20-35% over the weight of the boiled-off silk. The silk is then brought into

a lead-metal salt bath of di-chloride of lead,  $PbCl_2$ , of about 6° Bé. strength to which has been added 15% of decinormal sodium acetate,  $NaC_2H_3O_2 \cdot 3H_2O$ , in order to assist in holding the lead-metal salt in solution, and which has received a further acid concentration by the addition of 10% tri-basic phosphoric acid con.,  $H_3PO_4$ , and 5% isopropylated beta naphtha-line di-sulphonic acid which acts as a colloid. Although sodium acetate is desirable, it is not essential for the purpose of the invention. The treatment lasts for about 30 minutes and the temperature of the bath is maintained at 150° F. In order to neutralize the silk after the above treatment and to improve the fixation of the lead-metal salt, a bath in aqueous alkali, such as a 10% solution of ammonia carbonate,  $NH_4 \cdot HCO_3$ , is recommended. After this step the usual sodium silicate treatment of 3° Bé. strength at 45° C. is applied. The silk is then ready for soaping and dyeing.

The phosphoric acid used in the bath fulfills two distinct functions. First it serves as the producer of the needed high acid concentration which prevents undesirable precipitation on the fiber or in the bath itself, and secondly as the medium to produce the necessary phosphate-metal salt for the fixing of the lead compound on the fiber.

The fibroin of the silk undergoes a chemical change due to the high acid concentration in the lead-metal salt treatment, and forms a homogeneous compound with the tri-basic phosphate— $Pb_3(PO_4)_2$  produced in the bath, and the stannic acid-phosphate— $SnH_3PO_4$ —previously deposited in the interior of the fiber by the tin-phosphate treatment, the compound having the empirical formula  $Pb_3.Sn.(PO_4)_2 \cdot CH_3(NH)_2COOH$  etc.

It is also possible to use instead of phosphoric acid and sodium acetate in the lead-metal salt bath, di-sodium and tri-sodium phosphate with an increased amount of sodium acetate, or to increase the acid concentration of the bath by adding formic or mono-chloracetic acid, with or without the presence of sodium acetate.

For the protection of the fiber against the tendering influence of the strongly acid bath, an addition of colloids thereto is recommended, such as isopropylated beta naphtha-line di-sulphonic acid. These colloids can also be applied to the tin-weighted silk before entering into the lead bath, and not only protect the fiber, but also assist in preventing undesirable precipitation in the bath itself or on the fiber. In this case the addition of the colloid to the weighting bath may be dispensed with.

It is also possible to treat the silk before entering into the lead-metal solution with acids, such as formic or mono-chloracetic acid, or with salts which will induce the solubility of lead di-chloride in water, such as

sodium acetate, and to make this pre-treatment in the presence of protective colloids. The acid concentration of the lead-metal bath may then be diminished. In these cases a change of the silk fiber takes place which promotes a more equal absorption of the lead-metal salt.

If the tin-weighted silk is treated in a bath of proper proportions and temperatures according to the directions given above, the silk is heavily weighted with lead-metal compounds in a very short time. The precipitation-reaction necessary in the weighting process does not take place in the bath on account of the high acid content, but occurs in the interior of the fiber. It is possible to obtain from 25-60% gain in weight by a single immersion.

An added advantage of this process is the possibility to carry on the weighting of piece-goods in so-called jiggers, where the fabrics are treated in full width. As the weighting-reaction takes place very quickly, a single immersion will be found sufficient.

The result of the process described is a composite fiber consisting in a minor part of the fibroin of the silk and in a major part of the compound of tin, lead and phosphoric acid, homogeneously combined and which will give off none of its elementary component parts when treated with acetic acid or any other liquid with which the silk may come in contact during dyeing and finishing operations or when being worn and exposed to perspiration and other secretions of the human body.

I claim:

1. The process of weighting natural and artificial silk fiber which comprises treating said fiber in separate baths with tin-weighting agents and fixing baths, subsequently treating the fiber with aqueous solutions containing sodium acetate with isopropylated beta naphthaline di-sulphonic acid, and with di-chloride of lead in the presence of at least one material selected from the group consisting of phosphoric acid, di-sodium phosphate and tri-sodium phosphate, and finally treating said fiber in a bath of aqueous carbonate of ammonia.

2. The process of weighting natural and artificial silk fiber which comprises treating said fiber in separate baths with tin-weighting agents and fixing baths, subsequently treating the fiber with aqueous solutions containing sodium acetate and at least one acid from a group consisting of formic acid and mono-chlor-acetic acid with isopropylated beta naphthaline di-sulphonic acid, and with di-chloride of lead in the presence of at least one material selected from the group consisting of phosphoric acid, di-sodium phosphate and tri-sodium phosphate, and finally treating said fiber in a bath of aqueous carbonate of ammonia.

3. The process of weighting natural and

- artificial silk fiber which comprises treating said fiber in separate baths with tin-weighting agents and fixing baths, subsequently treating the fiber with aqueous solutions containing at least one acid from a group consisting of formic acid and mono-chloracetic acid with isopropylated beta naphthaline di-sulphonic acid, and with di-chloride of lead in the presence of at least one material selected from the group consisting of phosphoric acid, di-sodium phosphate and tri-sodium phosphate, and finally treating said fiber in a bath of aqueous carbonate of ammonia.
4. The process of weighting natural and artificial silk fiber which comprises treating said fiber in separate baths with tin-weighting agents and fixing baths, subsequently treating the fiber in a single bath containing di-chloride of lead, isopropylated beta naphthaline di-sulphonic acid, and sodium acetate in solution with at least one material selected from a group consisting of phosphoric acid, di-sodium phosphate, and tri-sodium phosphate, and treating said fiber in a bath of aqueous carbonate of ammonia.
5. The process of weighting natural and artificial silk fiber in separate baths with tin weighting agents and fixing baths, subsequently treating the fiber in a single bath containing di-chloride of lead, isopropylated beta naphthaline di-sulphonic acid in solution with an acid selected from a group consisting of formic acid and mono-chlor-acetic acid, and with at least one material selected from a group consisting of phosphoric acid, di-sodium phosphate and tri-sodium phosphate, and treating said fiber in a bath of aqueous carbonate of ammonia.
6. The process of weighting natural and artificial silk fiber in separate baths with tin weighting agents and fixing baths, subsequently treating the fiber in a single bath containing di-chloride of lead, isopropylated beta naphthaline di-sulphonic acid in solution with sodium acetate and an acid selected from a group consisting of formic acid and mono-chlor-acetic acid, and with at least one material selected from a group consisting of phosphoric acid, di-sodium phosphate and tri-sodium phosphate, and treating said fiber in a bath of aqueous carbonate of ammonia.
7. The process of weighting natural and artificial silk fiber which comprises treating said fiber in separate baths with tin-weighting agents and fixing baths, subsequently treating the fiber with aqueous solutions containing sodium acetate with a colloid, and with di-chloride of lead in the presence of at least one material selected from the group consisting of phosphoric acid, di-sodium phosphate and tri-sodium phosphate, and finally treating said fiber in a bath of aqueous alkali.
8. The process of weighting natural and artificial silk fiber which comprises treating said fiber in separate baths with tin-weighting agents and fixing baths, subsequently treating the fiber with aqueous solutions containing sodium acetate and at least one acid from a group consisting of formic acid and mono-chlor-acetic acid with a colloid, and with di-chloride of lead in the presence of at least one material selected from the group consisting of phosphoric acid, di-sodium phosphate and tri-sodium phosphate, and finally treating said fiber in a bath of aqueous alkali.
9. The process of weighting natural and artificial silk fiber which comprises treating said fiber in separate baths with tin-weighting agents and fixing baths, subsequently treating the fiber with aqueous solutions containing at least one acid from a group consisting of formic acid and mono-chlor-acetic acid with a colloid, and with di-chloride of lead in the presence of at least one material selected from the group consisting of phosphoric acid, di-sodium phosphate and tri-sodium phosphate, and finally treating said fiber in a bath of aqueous alkali.
10. The process of weighting natural and artificial silk fiber which comprises treating said fiber in separate baths with tin-weighting agents and fixing baths, treating said fiber in an aqueous bath containing a material selected from the group consisting of formic acid and mono-chlor-acetic acid in solution with isopropylated beta naphthaline di-sulphonic acid, and in another subsequent aqueous bath containing di-chloride of lead in the presence of at least one material selected from a group consisting of phosphoric acid, di-sodium phosphate, and tri-sodium phosphate, and finally treating said fiber in a bath of aqueous carbonate of ammonia.
11. The process of weighting natural and artificial silk fiber which comprises treating said fiber in separate baths with tin-weighting agents and fixing baths, treating said fiber in an aqueous bath containing a material selected from the group consisting of formic acid and mono-chlor-acetic acid in solution with isopropylated beta naphthaline di-sulphonic acid, and in another subsequent aqueous bath containing di-chloride of lead and sodium acetate in the presence of at least one material selected from a group consisting of phosphoric acid, di-sodium phosphate, and tri-sodium phosphate, and finally treating said fiber in a bath of aqueous carbonate of ammonia.
12. The process of weighting natural and artificial silk fiber which comprises treating said fiber in separate baths with tin-weighting agents and fixing baths, treating said fiber in an aqueous bath containing sodium acetate in solution with isopropylated beta naphthaline di-sulphonic acid, and in another subsequent aqueous bath containing di-chloride of lead.

of lead in the presence of at least one material selected from a group consisting of phosphoric acid, di-sodium phosphate, and tri-sodium phosphate, and finally treating said fiber in a bath of aqueous carbonate of ammonia.

13. The process of weighting natural and artificial silk fiber which comprises treating said fiber in separate baths with tin-weighting agents and fixing baths, treating said fiber in an aqueous bath containing sodium acetate and a material selected from the group consisting of formic acid and mono-chlor-acetic acid in solution with isopropylated beta naphthaline di-sulphonic acid, and in another subsequent aqueous bath containing di-chloride of lead in the presence of at least one material selected from a group consisting of phosphoric acid, di-sodium phosphate, and tri-sodium phosphate, and finally treating said fiber in a bath of aqueous carbonate of ammonia.

14. A step in the weighting process of natural and artificial silk fiber which comprises the treatment of the fiber in a single bath comprising lead di-chloride, a colloid, and a material selected from a group consisting of phosphoric acid, di-sodium phosphate and tri-sodium phosphate.

15. A step in the weighting process of natural and artificial silk fiber which comprises the treatment of the fiber in a single bath comprising lead di-chloride, sodium acetate, a colloid, and a material selected from a group consisting of phosphoric acid, di-sodium phosphate and tri-sodium phosphate.

16. A step in the weighting process of natural and artificial silk fiber which comprises the treatment of the fiber in a single bath comprising lead di-chloride, a material selected from a group consisting of formic acid and mono-chlor-acetic acid, a colloid, and a material selected from a group consisting of phosphoric acid, di-sodium phosphate and tri-sodium phosphate.

17. A step in the weighting process of natural and artificial silk fiber which comprises the treatment of the fiber in a single bath comprising lead di-chloride, sodium acetate, a material selected from a group consisting of formic acid and mono-chlor-acetic acid, a colloid, and a material selected from a group consisting of phosphoric acid, di-sodium phosphate and tri-sodium phosphate.